

F. A. KRAFT.

Zincing Bath.

No. 79,234.

Patented June 23, 1868.

*Fig. 1.*



*Fig. 2.*



Witnesses:

Wm. A. Steel.

John Parker.

Inventor:

F. Kraft  
By his Atty  
J. H. Lawson

# United States Patent Office.

FREDERICK A. KRAFT, OF PHILADELPHIA, PENNSYLVANIA.

*Letters Patent No. 79,234, dated June 23, 1868.*

## IMPROVEMENT IN ZINCING IRON.

The Schedule referred to in these Letters Patent and making part of the same.

TO ALL WHOM IT MAY CONCERN:

Be it known that I, FREDERICK A. KRAFT, of Philadelphia, Pennsylvania, have invented an Improved Zincing-Bath; and I do hereby declare the following to be a full, clear, and exact description of the same.

My invention relates to the zincing of articles of iron or other metal, by immersing them in molten zinc; and my invention consists of a zincing-bath composed of an outer casing of iron lined with copper or equivalent material, for preventing the formation of a dross from the iron and zinc, which tends to destroy the iron vessel, and renders a great portion of the zinc unfit for coating purposes.

I will now proceed to describe a mode of carrying the same into effect, reference being had to the accompanying drawing, which forms a part of this specification, and in which—

Figure 1 represents a portion (full sized) of a zincing-bath.

Figure 2, a transverse section of the bath, drawn to a reduced scale of one inch to a foot.

In conducting the process of coating iron with zinc, it has been usual to employ cast or wrought-iron vessels for containing the zinc, which is maintained in a molten condition by the application of external heat.

Vessels of the smaller size are occasionally made of cast iron, but those of larger size of thick wrought-iron plates.

For a vessel twelve feet long, twenty-six inches wide, and forty inches deep, for instance, wrought-iron plates one inch in thickness are necessary, to withstand the pressure of the zinc, a coke fire contained in a recess continued on all sides of the vessel, being used for maintaining the zinc at or about the temperature of 750° Fahrenheit.

Owing to the intimate contact of the zinc with the iron, and to the heat to which both are subjected, the two metals oxidize rapidly, forming what is known as "spelter-dross," which settles on the bottom of the vessel, and the greater the heat the faster does this so-called dross accumulate.

The evils resulting from the formation of this dross in ordinary zincing-baths may be enumerated as follows:

First, the reduction of the zinc to the condition of dross, useless for coating purposes, and of half the value of the pure zinc, to the condition of which it cannot be restored without resorting to tedious and expensive processes.

Second, the rapid destruction of costly wrought-iron vessels; and

Third, the tedious manipulation demanded in removing the dross from the pure zinc.

In order to obviate these evils, I line the cast or wrought-iron vessel with a material which, at the temperature to which it is usually subjected, will not be affected by or form an alloy with the zinc, or which will not so readily form an alloy with the latter as iron.

In fig. 1, of the drawing, A represents a portion of the outer casing of wrought iron, and B a thin lining of copper, riveted to the outer casing at suitable intervals.

It is not necessary, in order to maintain the zinc in a proper molten condition, to heat it above 750° or 800°, and as at this temperature no combination can be effected between copper and zinc, the formation of dross, in a vessel lined with copper or equivalent material, cannot take place.

Through carelessness, however, the vessel may be heated to such an extent that the copper would form an alloy with the zinc; but as a provision against such accidents, the surface of the copper exposed to the zinc may have a thin coating of silver, which, although it can be melted at a less heat than copper, has not such an affinity as the latter for zinc.

The interior of the vessel may be lined with thin fire-tiles in place of copper, the tiles being secured by copper or other fastenings, or slabs of slate, or glass or earthenware may be used for lining-purposes, with good results as regards preventing the formation of the above-mentioned dross; or the interior of the vessel may be lined at the sides with copper, and at the bottom with fire-tiles, slate, glass, &c.

I claim as my invention, and desire to secure by Letters Patent—

A zincing-bath, composed of an outer casing of iron, containing an inner lining or casing of copper or its equivalent, as set forth.

In testimony whereof, I have signed my name to this specification in the presence of two subscribing witnesses.

FRED. A. KRAFT.

Witnesses:

W.M. A. STEEL,  
HARRY SMITH.